

## UNITED STATES PATENT OFFICE

2,295,844

## PROCESS OF SPINNING CUPRAMMONIUM CELLULOSE SOLUTIONS

Franz Hoelkeskamp and Ewald Knehe, Wuppertal-Barmen, Germany; vested in the Alien Property Custodian

No Drawing. Application January 18, 1940,  
Serial No. 314,562. In Germany January 18,  
1939

4 Claims. (Cl. 18—54)

This invention relates to improvements in methods for producing artificial silk by the cuprammonium stretch-spinning process.

It is an object of the invention to provide a method for producing filaments, fibres, threads and the like from cuprammonium cellulose solutions, using the so-called stretch-spinning process and which is immune from drawbacks created by variations in the amount of spinning water used and by fluctuations in the temperature at which the spinning of the filaments is effected.

It is a further object of the invention to provide a method whereby cuprammonium artificial silk can be obtained which will possess a uniform hand, and uniform dye affinity despite variations in the manufacturing factors recited above.

To this end the invention is based on the use of means for causing the freshly spun filaments, threads and the like to adsorb negative ions of alkali metal silicates, such adsorption being suitable for producing filaments and threads of uniform hand and uniform dye affinity despite the above recited variations in the manufacturing conditions.

In the manufacture of fibres and threads, such as those made of artificial silk, staple fibres, and the like, from cuprammonium cellulose solutions by the stretch-spinning method, the uniformity of the products obtained depends to a great extent upon the uniformity with which the threads are hardened in the spinning funnel and the latter factor in turn upon the accurate measurement of the quantity of water used in the spinning process as well as the accurate maintenance of the spinning temperature at which operations are conducted.

Variations in the amount of water used and fluctuations in the spinning temperature serve to produce products of non-uniform hand (that is, products having a non-uniform degree of softness). Such lack of uniformity results in the production of a non-uniform mesh when the products are subsequently worked up into finished goods as well as unevenness when the spun or subsequently woven products are dyed. Thus, a drop in the spin water temperature imparts a harder hand to the goods and consequently leads to the production of an irregular mesh when the material is worked up.

The present invention makes it possible to render the spinning process immune from these drawbacks, that is, from the deleterious results accruing from the practically unavoidable variations in the amount of spinning water and the fluctuations in the spinning temperature. It has

been found that the addition to the spinning water of small quantities of water-soluble an alkali metal silicate produces an astonishing effect in this direction. Both the hand (that is, the degree of softness) as well as the dyeing capacity become most exceptionally and uniformly regulated through adoption of this measure notwithstanding variations in spinning water quantity and temperature.

Among the substances which are adapted to produce the results desired, a preferred one is ordinary sodium silicate which is preferably used in the form of waterglass. By way of describing the practice of the invention, therefore, an executive example is given herewith, it being understood that the use of waterglass is merely illustrative and that other alkali metal silicates may be used:

20 A comparison control sample of skein silk of 120 denier strength was produced on an ordinary production machine for cuprammonium cellulose solutions using a quantity of spinning water amounting to 725 c. c. per minute, at a temperature of 35° C., but without using any addition of waterglass; the material was then finished up in the usual manner.

25 By way of comparison, a skein silk of 120 denier strength was produced in the same spinning machine from the same cellulose solution and using 30 the same quantity of spinning water with the exception that 200 mg. per liter of an alkali metal silicate, such as sodium waterglass were added. The product was then worked up in an analogous manner.

35 As regards the products obtained, it was found that those produced with the aid of the waterglass addition were in every possible manner far more uniform than those produced without the use of waterglass in the spinning water. This 40 fact was readily established with the aid of suitable testing apparatus, the tests being directed towards evaluating the hand or degree of softness. The products spun with the aid of waterglass were relatively soft, and, when judged according to their measured degree of softness, 45 could be classified in a narrowly defined range of values. In other words they were substantially uniform in quality. The products spun without the use of waterglass however exhibited appreciable variations and erratic measurement values when evaluated as to softness, so that numerous strands thereof were found to be relatively hard in some parts and again quite soft in others.

50 It was found that if the two products made in

accordance with the executional and comparison example given above, are worked up, say into stocking lengths, the strands that were produced with the aid of a waterglass produced a uniform mesh structure, whereas the analogous stocking strands made from skeins produced without the use of a waterglass exhibited very appreciable detectable variations in the mesh structure. A dyeing capacity test also served very clearly to bring out the advantage of adding a waterglass to the spinning water.

The advantageous effects secured by adding a waterglass was also very clearly perceptible if, for example, while using the same quantity of spinning water (725 c. c. per minute) different spinning water temperatures were deliberately used, say, temperatures of 35°, 28°, 24°, and 21°, and if 200 mg. of sodium waterglass were added to the spinning water. In the instances where a waterglass was added, the differences in the qualities of the produced threads or fibres became practically equalized despite the great differences in the spinning water temperatures. However, if the water glass was omitted, very great differences in quality were produced. With a spinning water conditioned to 35°, a soft material was obtained but the products became increasingly "harder" as the spinning water temperature decreased; furthermore, they exhibited an unsatisfactory mesh formation and uneven dyeing capacity. Heretofore it had been impossible for many practical purposes in manufacturing a given woven article to use a plurality of artificial silk batches produced under spinning conditions where such varying temperatures had prevailed.

The quantities of the substances embraced by the present invention and that are to be added depends upon various factors and may vary within wide limits. The layout of the spinning room, and the ventilation and air conditioning thereof all tend to increase or decrease the danger of producing fluctuations in the temperature of the spinning water in the various individual spinning funnels, and these factors will govern the advisability of including larger or smaller quantities of the addi-

tion agents in the total spinning water involved. The same is true concerning variations in the quantity of spinning water that has to be reckoned with. Under certain circumstances and conditions, quantities as small as 30 or 50 mg. per liter of addition agents may render satisfactory service, whereas in other cases 100, 200 and even 500 mg. per liter may be required.

What is claimed is:

1. In the method of producing filaments, fibres, threads and the like having a uniform hand and dye affinity from cuprammonium cellulose spinning solutions by the stretch-spinning process, the step which comprises spinning a cuprammonium cellulose solution into water containing about 30-500 milligrams per liter of an alkali metal silicate, said water having a temperature of about 21-35° C.

2. In the method of producing filaments, fibres, threads and the like having a uniform hand and dye affinity from cuprammonium cellulose spinning solutions by the stretch-spinning process, the step which comprises spinning a cuprammonium cellulose solution into water containing about 30-500 milligrams per liter of sodium silicate, said water having a temperature of about 21-35° C.

3. In the method of producing filaments, fibres, threads and the like having a uniform hand and dye affinity from cuprammonium cellulose spinning solutions by the stretch-spinning process, the step which comprises spinning a cuprammonium cellulose solution into water containing about 200 milligrams per liter of an alkali metal silicate, said water having a temperature of about 35° C.

4. In the method of producing filaments, fibres, threads and the like having a uniform hand and dye affinity from cuprammonium cellulose spinning solutions by the stretch-spinning process, the step which comprises spinning a cuprammonium cellulose solution into water containing about 200 milligrams per liter of sodium silicate, said water having a temperature of about 21-35° C.

FRANZ HOELKESKAMP.  
EWALD KNEHE.